

## UNITED STATES PATENT OFFICE

ROBERT S. ARCHER AND WILLIAM L. FINE, OF CLEVELAND, OHIO, ASSIGNORS TO ALUMINUM COMPANY OF AMERICA, OF PITTSBURGH, PENNSYLVANIA, A CORPORATION OF PENNSYLVANIA

## METHOD OF TREATING ALUMINUM BASE ALLOYS WHICH ARE SUBJECT TO GROWTH

No Drawing. Application filed December 22, 1928. Serial No. 328,048.

The invention relates to the treatment of aluminum base alloys which undergo permanent increases in volume when heated. While particularly applicable to the treatment of pistons and other aluminum base alloy articles which are used as parts, either moving or fixed, of internal combustion engines and the like, in its broader aspects the invention applies to the treatment of all kinds 5 of articles used under various conditions where increases in their volumes are undesirable, and which are formed of aluminum base alloys of the type explained.

It is well known that some aluminum base 15 alloys, when subjected to elevated or even slightly elevated temperatures, undergo a gradual and permanent increase in volume which finally attains a maximum, while other such alloys are not so characterized even when 20 held at elevated temperatures for an extended period of time. At present, actual experiment is necessary to determine whether a particular aluminum base alloy will or will not undergo this permanent increase in 25 volume, there being no reliable means of predicting it. This increase in volume is different in nature from the thermal expansion of a metal in which an equal contraction occurs on cooling, and the phenomenon has been designated as "growth" or "permanent growth", 30 and is so designated herein.

The fact that some aluminum base alloys grow when subjected to elevated temperatures, by which is meant here and throughout 35 this specification temperatures not greatly exceeding 350° C. has long been recognized as a disadvantage which in many cases should be overcome before the alloys are satisfactory for uses where their retention of original dimensions is an important factor. To 40 preclude growth in finished articles, thermal methods have been devised by which growth is fully developed before the articles are finally shaped to finished dimensions. Usually 45 the method consists in heating the alloys to a temperature of from about 275° to 450° C. for a period of time, customarily varying between one to ten hours, or until maximum 50 growth is obtained. To the best of our

knowledge this is the only method which has been commercially used for this purpose.

Because of the relatively high temperatures used, this method has the serious disadvantage of softening the alloys because 55 they lose a substantial portion of their hardness when heated for considerable periods of time at the above mentioned temperatures, within the stated range of which is usually found the commercial annealing temperature 60 of the particular alloy being treated, or in other words the temperature at which the alloy can be most efficiently softened. Consequently, aluminum base alloys in which maximum volume changes have been developed by thermal treatments from about 65 275° to 450° C. have usually lost substantially proportions of their original or attainable hardness.

Satisfactory methods of developing maximum growth in aluminum base alloys are of considerable importance for many uses of the articles of which they are formed, but in no field of industrial application has the necessity of developing maximum growth as 70 yet become so important as in the case of aluminum base alloy pistons. The conditions of service of such pistons make the hardness of the alloys, and their ability to maintain required dimensions, properties of great 75 importance; and the substantial decrease in importance; and the substantial decrease in hardness caused by the prevailing practice in heating the alloys to obtain maximum growth has considerably detracted from the peculiar usefulness of the alloys as materials 80 for the manufacture of pistons.

The object of the invention is to provide a method of thermal treatment of aluminum base alloys which grow, whereby maximum growth of the alloys may be effected without 85 a simultaneous substantial decrease in hardness, and which method is simple, effective and practical for treating aluminum base alloy pistons and other articles in which hardness is important.

The invention is predicated upon our discovery that substantially complete or maximum volume change may be developed in aluminum base alloys subject to growth by heating the alloys to temperatures of from 90 95 100

about 150° to 265° C. and continuing the heating until the hardness of each alloy has passed through its maximum and the alloy has attained a substantially complete and 5 permanent increase in volume. Although it has heretofore been considered that these temperatures are too low for such treatment, we have found that, after adequate treatment at them, aluminum base alloys do not undergo 10 further growth in service.

In the practice of the invention, the selection of a particular treating temperature depends upon the aluminum base alloy to be treated and its desired final hardness. In 15 general, the lower temperatures of treatment produce higher hardnesses at maximum growth. Within the temperature range of about 150° to 265° C. a considerably higher hardness is attained at the point of maximum 20 growth than obtained by the prior processes, and, when maximum hardness is desired, it is preferred to use a temperature of from 150° to 185° C. As to time, that required to obtain maximum growth depends to a large 25 extent upon the temperature used, and to a lesser extent upon the aluminum base alloy to be treated. The nature of one such alloy as compared with another may be such as require considerable variation of the period of 30 heating at any given temperature, but for any one aluminum base alloy the time of heating necessary to develop maximum growth is shorter the higher the temperature, as will presently appear from examples which will 35 be given.

To further an understanding of our invention it seems desirable to first explain the manner in which certain well known heat treatable aluminum base alloys respond to 40 heat treatment to produce structural changes in them. Such heat treatment usually comprises three steps, namely, a solution heat treatment, a rapid cooling or quenching to ordinary room temperature, and an aging 45 treatment. The solution heat treatment consists in heating a so-called heat-treatable alloy to a temperature slightly below the eutectic temperature, or the temperature of incipient fusion of the alloy, for a period of 50 time sufficient to place a substantial part of the undissolved soluble alloying constituents in solid solution with the aluminum. The second or cooling step consists in rapidly 55 cooling the alloy from its solution heat treatment to retain at ordinary temperature the solid solutions formed during the solution treatment. The third or aging treatment causes the unstable solid solutions thus retained to break down in such a manner that 60 the hardness and tensile strength of the alloy is increased, which increase in hardness and strength is probably caused by the precipitation of dissolved constituents from the solid solution. The aging treatment is usually effected by heating the alloy to a relatively low 65

temperature for such period of time as is necessary to develop the most favorable combination of hardness and strength, and in practice this time does not exceed the point at which the strength of the alloy has become 70 maximum and its hardness has approached a maximum. Continuation of ageing causes the strength and hardness to pass through their respective maxima, and to subsequently decrease, over-aging having been considered 75 undesirable because it produces less than maximum strength and hardness.

In working with heat treatable aluminum base alloys we have discovered that their solution heat treatments decrease their volumes 80 as compared with those as cast, and that the aging treatments, and also thermal treatments at considerably higher temperature than the aging treatments, increase their volumes as compared to those as cast. In the light of what is known and believed concerning the structural changes which take place in aluminum base alloys during heat treatments, we have come to the conclusion that their volume changes are caused by either 85 the solution, in the case of decreased volume, or the precipitation, in the case of increased volume, of the soluble alloying constituents. Accordingly, the phenomenon of growth in aluminum base alloys may be attributed to 90 the difference in volume between an alloying constituent as it is present in solid solution in aluminum, and as it is present in the undissolved or precipitated condition. Thus, 95 an aluminum base alloy which has been submitted to a solution heat treatment, or is in the as cast and untreated condition, contains 100 a certain amount of alloying constituent held in a solid solution with the aluminum, which, when the alloy is subjected to certain elevated temperatures, tends to precipitate from the solid solution in a form which in volume 105 is larger than the volume of the same constituent in solid solution, causing the alloy to increase in volume, or, in other words, to 110 grow. The magnitude of this increase in volume is affected by the size and distribution 115 of the precipitated particles. While we believe this explanation to be correct, it will be understood that the theory is merely explanatory, and that it is not limiting upon the scope of the appended claims.

As above mentioned, we have discovered the heretofore unrecognized fact that maximum growth can be developed at materially 120 lower temperatures than heretofore used without the substantial loss in hardness which attends the prior growth-developing treatment. We have also discovered that by these low temperature treatments full growth 125 cannot be obtained unless the treatment is extended beyond the point where maximum hardness and strength is developed, with respect to which our process differs in substance 130 from the aging treatments which have been

and are being used for the development of strength and hardness in heat treatable aluminum base alloys, and which have been practically limited to temperatures of from 5 about 100° to 200° C. to attain their intended purposes. The method herein provided, and which as stated may be practiced with good results at temperatures from about 150° to 265° C. contemplates the development of 10 maximum growth in the alloys, and is therefore continued beyond the point of maximum hardness to the point of maximum growth. Although in obtaining maximum growth the hardness of an alloy is developed to a maximum 15 and then decreased, the hardness finally retained by the alloy is much greater than the hardness of the alloy after being subjected to the prior growth-developing treatments at temperatures from about 275° to 20 450° C. and the alloy is sufficiently hard for the service conditions of pistons or other articles where both hardness and the elimination of changes in volume are factors of prime importance.

25 By way of example, the advantages of this invention over the prior practice are illustrated by the results produced on two chill cast pistons formed of aluminum base alloys containing 10% copper as the main alloying constituent, each of which pistons was given a solution heat treatment at 495° C. and quenched in water. One of these pistons was then subjected to a growth-developing treatment consisting of heating it at 375° C. 30 until maximum growth was obtained, after which the piston had a Brinell hardness of 61 and a unit growth per inch of 0.00022, of an inch. The other piston was subjected to a growth-developing treatment according to 35 this invention by heating it at a temperature of 225° C. until full growth was obtained, after which the piston had a Brinell hardness of 121 and a unit growth per inch of 0.00091 of an inch.

40 As examples of the various temperatures that may be used in, and the various times required for, practicing the growth-developing treatment herein provided, a chill cast aluminum-copper alloy piston required a heating period of 200 hours at 154° C. before 45 maximum growth was obtained, the Brinell hardness of the piston then being 142. Another chill cast piston made from the same alloy required only 86 hours at 170° C. to 50 develop maximum growth, its Brinell hardness then being 142, while a third chill casting of the same alloy required 19 hours heating at 225° C. to develop maximum growth, its Brinell hardness then being 120. In all of 55 these cases a growth per inch of 0.0006 of an inch was obtained, and with further heating no additional measurable growth took place.

60 It is apparent from these examples that, because of the short heating period, a treatment at 225° C. is better adapted to commer-

cial practice than, for example, a treatment at 154° C. However, when as a governing factor the highest obtainable hardness is required at the point of maximum growth, the longer heat treatments at lower temperatures may be economically feasible. The hardness developed in each of the foregoing examples is considerably higher than that developed by the prior treatments, and the Brinell hardness of 120 produced by a treatment for 19 hours at 225° C. is sufficiently high for 70 most purposes.

75 As further examples of the practice of our invention, a chill cast aluminum base alloy containing 7% copper, 7% silicon, 7½% nickel and 0.58% iron, obtained its maximum growth after being heated for 22 hours at 225° C. Its Brinell hardness was then 114, and it had a unit growth per inch of 0.00091 of an inch. Another aluminum base alloy containing 14% silicon 2% nickel, 1% magnesium and 0.75% copper cast in the form of a piston was given a solution heat treatment and subsequently heated for 17 hours at 225° C. at which time its maximum growth was obtained. The piston then had a Brinell hardness of 107 and a unit growth per inch of 0.00028 of an inch. Still another aluminum base alloy containing 4% copper and 2% nickel cast in the form of a piston was given a solution heat treatment at 535° C. for 16 hours and quenched in water, after which it had a Brinell hardness of 60. This piston was then heated for 36 hours at 225° C. when its full growth was obtained, and it then had a Brinell hardness of 80 and a unit growth per inch of 0.00075 of an inch.

90 These examples illustrate the applicability of our invention to various commercial aluminum base alloys by heat treating them at a temperature of 225° C. and from the examples it will be observed that the nature of the alloy determines the length of time required to reach the point of maximum growth. However, in every case the point of maximum growth is reached by a treatment 95 extending for an appreciable time beyond that required for attaining maximum hardness, for otherwise maximum growth cannot be obtained.

100 According to the provisions of the patent statutes, we have explained the principle and mode of operation of our invention, and have given several specific examples of the way in which it may be practiced. However, we desire to have it understood that, within the scope of the appended claims, the invention may be practiced otherwise than according to the specific examples, and that its beneficial results extend to aluminum base alloys 105 which are subject to growth other than those of the specific examples.

110 We claim as our invention:

115 1. The method of developing substantially complete and permanent volume change in 120

70

75

80

85

90

95

100

105

110

115

120

125

130

an aluminum base alloy which is subject to growth, comprising heating the alloy to a temperature of from about 150° to 265° C. and continuing said heating until the hardness of the alloy has passed through its maximum and the alloy has attained a substantially complete and permanent increase in volume:

5 2. The method of developing substantially complete and permanent volume change in an aluminum base alloy containing copper and which is subject to growth when heated, comprising heating the alloy to a temperature of from about 150° to 265° C. and continuing 75  
15 said heating until the hardness of the alloy has passed through its maximum and the alloy has attained a substantially complete and permanent increase in volume.

20 3. The method of developing substantially complete and permanent volume change in an aluminum base alloy containing copper and silicon and which is subject to growth when heated, comprising heating the alloy to a temperature of from about 150° to 265° C. 80  
25 and continuing said heating until the hardness of the alloy has passed through its maximum and the alloy has attained a substantially complete and permanent increase in volume.

30 4. The method of developing substantially complete and permanent volume change in an aluminum base alloy which is subject to growth, comprising heating the alloy to a temperature of from about 150° to 185° C. 85  
35 and continuing said heating until the hardness of the alloy has passed through its maximum and the alloy has attained a substantially complete and permanent increase in volume.

40 5. The method of developing substantially complete and permanent volume change in a piston formed of an aluminum base alloy which is subject to growth, comprising heating the piston to a temperature of from about 45 150° to 265° C. and continuing said heating until the hardness of the alloy of which it is formed has passed through its maximum and the alloy has attained a substantially complete and permanent increase in volume. 100  
50

55 6. An article of manufacture formed of an aluminum base alloy which is subject to growth, said article having a Brinell hardness of not less than about 80 and a structure obtained when the alloy is heated to a temperature of from about 150° to 265° C. until its hardness has passed through its maximum and the alloy has attained a substantially complete and permanent increase in volume. 110  
60

65 7. A piston formed of an aluminum base alloy which is subject to growth, said piston having a Brinell hardness of not less than about 80 and a structure obtained when the alloy of which it is formed is heated to a temperature of from about 150° to 265° C. until its hardness has passed through its maximum 120  
65

and the alloy has attained a substantially complete and permanent increase in volume. In testimony whereof, we hereunto sign our names.

ROBERT S. ARCHER. 70  
WILLIAM L. FINK.

75

80

85

90

95

100

105

110

115

120

125

130